

July 30, 1940.

A. C. G. EGERTON

2,209,646

METHOD OF PREVENTING THE FORMATION OF GUMLIKE PRODUCTS IN OILS

Filed June 29, 1938



Inventor:  
Alfred Charles Glyn Egerton,  
By  
Stebbins, Blenko & Parmelet,  
attys.

## UNITED STATES PATENT OFFICE

2,209,646

METHOD OF PREVENTING THE FORMATION  
OF GUMLIKE PRODUCTS IN OILS

Alfred Charles Glyn Egerton, London, England

Application June 29, 1938, Serial No. 216,595  
In Great Britain July 2, 1937

16 Claims. (CL 252—25)

This invention relates to a method of preventing the formation of gumlike products in oils which are subjected to an atmosphere containing oxides of nitrogen.

It was hitherto believed that the formation of gummy matter in oils was due to the oxidation of the oil leading directly to the production of gummy oxidation products. It has now been found, however, that the formation of gumlike products in an oil used in an engine operating at or near the detonation point is greater than when the engine is not operating under detonating conditions (see Egerton, Smith & Ubbelohde, Royal Society of London "Philosophical Transactions, 1935," vol. 234, page 433). In an engine operating under detonating conditions it was also shown, in the above publication, that the amounts of nitrogen oxides formed in the combustion chamber were abnormal.

It has now been found that the oxide of nitrogen which has the greatest effect in promoting the formation of gums is nitrogen peroxide.

It is an object of this invention to minimise the effect of the nitrogen peroxide on the oil by the addition thereto of a nitrogen oxide inhibitor which acts either by stopping or reducing the catalytic action of nitrogen peroxide or by absorbing nitrogen peroxide and converting it into a harmless compound.

A number of experiments have shown that when oil is maintained at a temperature of 218° C. and air containing nitrogen peroxide in a proportion of about 2 parts in  $10^4$  parts of air, the amount of gum formed is increased up to about ten times the amount formed when air alone is blown through the oil. These same experiments have shown that the presence of nitric oxide in the air does not increase the amount of gum formed as compared with the amount formed when air alone is used.

According to this invention a method of preventing the formation of gumlike products in oil subjected to an atmosphere containing oxides of nitrogen consists in introducing into said oil or said atmosphere a small proportion of a ferric compound. That is to say, the small proportion of the ferric compound may be introduced directly into and dispersed in said oil; or, instead, said ferric compound may be introduced into said atmosphere to which the oil is subjected by introduction, either separately from or in dispersion in the motor fuel, into the combustion chamber of the internal combustion engine with which said oil is used. The last mentioned practice, the introduction of the ferric compound into

the combustion chamber of the engine in dispersion in the engine fuel, presents the advantage of the use of the ferric inhibitors of the present invention commercially as additions to the gasoline or other like fuel of an internal combustion engine for the purpose of minimizing the effect of nitrogen peroxide on the lubricating oil under operating conditions of the engine.

Oxidation tests which have been carried out have shown that the addition of small quantities of ferric oxide markedly reduce the amount of gum formed in an oil which is heated in the presence of nitrogen peroxide, and it is therefore a feature of the invention that ferric oxide is added to the oil.

The use of ferric salts of fatty acids has been found very considerably to reduce the formation of gum; ferric ricinoleate has been tested and found to be particularly successful.

The drawing shows a diagrammatic arrangement whereby the gum inhibitor may be introduced into the combustion chamber of an internal combustion engine and shows a tank of the gum inhibitor connected by a supply line to the engine communicating with the combustion chamber through which supply line the gum inhibitor is introduced into the combustion chamber.

I claim:

1. A lubricant comprising a lubricating oil adapted for use in an internal combustion engine and having dispersed therein a small proportion of an inorganic ferric compound adapted to retard or inhibit gum formation in said oil.

2. A lubricant comprising a lubricating oil adapted for use in an internal combustion engine and having dispersed therein between 0.5 and 5% by weight of an inorganic ferric compound adapted to retard or inhibit gum formation in said oil.

3. A lubricant comprising a lubricating oil having dispersed therein a small proportion of ferric oxide.

4. A lubricating oil adapted for use in an internal combustion engine and having dispersed therein between .05 and 5% by weight of ferric ricinoleate adapted to retard or inhibit gum formation in said oil.

5. A method of preventing the formation of gumlike products in lubricating oils subjected to the action of an atmosphere containing nitrogen peroxide in an internal combustion engine which consists in dispersing in the engine fuel a small proportion of a ferric salt of a fatty acid capable of functioning as a retarder or inhibitor of gum

formation in said oils subjected to said atmosphere.

6. A method of preventing the formation of 5  
gumlike products in lubricating oils subjected to  
the action of an atmosphere containing nitrogen  
peroxide in an internal combustion engine which  
consists in dispersing in the engine fuel a small  
proportion of ferric ricinoleate.

7. A method of preventing the formation of 10  
gumlike products in lubricating oils subjected to  
the action of an atmosphere containing nitrogen  
peroxide in an internal combustion engine which  
consists in introducing into the lubricating oil  
a nitrogen peroxide inhibitor of the class con- 15  
sisting of inorganic ferric compound, organic  
ferric compounds and ferric salts of fatty acids.

8. A method of preventing the formation of 20  
gumlike products in lubricating oils subjected to  
the action of an atmosphere containing nitrogen  
peroxide in an internal combustion engine which  
consists in introducing into the lubricating oil  
a nitrogen peroxide inhibitor comprising ferric 25  
oxide.

9. A method of preventing the formation of 30  
gumlike products in lubricating oils subjected to  
the action of an atmosphere containing nitrogen  
peroxide in an internal combustion engine which  
consists in introducing into the lubricating oil  
a nitrogen peroxide inhibitor comprising ferric 35  
ricinoleate.

10. A method of preventing the formation of 40  
gumlike products in lubricating oils subjected to  
the action of an atmosphere containing nitrogen  
peroxide in an internal combustion engine which  
consists in introducing into the lubricating oil  
a nitrogen peroxide inhibitor comprising ferric 45  
ricinoleate in the proportion of between .05 and  
5% by weight of the oil.

11. A motor fuel for an internal combustion 45  
engine using lubricating oil and subjecting said  
oil to an atmosphere of nitrogen peroxide in the  
engine tending to cause formation of gumlike  
products in said oil, said motor fuel comprising  
gasoline or the like combustible hydrocarbon  
having a small proportion of ferric oxide dis- 50  
persed therein.

12. A motor fuel for an internal combustion 5  
engine using lubricating oil and subjecting said  
oil to an atmosphere of nitrogen peroxide in the  
engine tending to cause formation of gumlike  
products in said oil, said motor fuel having a 10  
small proportion of ferric ricinoleate dispersed  
therein.

13. A method of preventing the formation of 15  
gumlike products in lubricating oils subjected to  
the action of an atmosphere of nitrogen peroxide 10  
in an internal combustion engine tending to cause  
such formation, which method comprises intro- 15  
ducing into the combustion chamber of the in-  
ternal combustion engine a small proportion of a  
ferric compound capable of functioning to retard 15  
or inhibit action of nitrogen peroxide in forma-  
tion of gumlike products in said oils subjected  
to said atmosphere.

14. A method of preventing the formation of 20  
gumlike products in lubricating oils subjected to  
the action of an atmosphere containing nitro- 20  
gen peroxide in an internal combustion engine  
tending to cause such formation, which method  
consists in dispersing in the engine fuel a small  
proportion of a ferric compound capable of func- 25  
tioning to retard or inhibit action of nitrogen  
peroxide in formation of gumlike products in said  
oils subjected to said atmosphere.

15. A method of preventing the formation of 30  
gumlike products in lubricating oils subjected to  
the action of an atmosphere containing nitrogen  
peroxide in an internal combustion engine which  
consists in introducing into the combustion 35  
chamber of the internal combustion engine a  
nitrogen peroxide inhibitor of the class consisting  
of inorganic ferric compounds, organic ferric  
compounds and ferric salts of fatty acids.

16. A method of preventing the formation of 40  
gumlike products in lubricating oils subjected to  
the action of an atmosphere containing nitrogen 40  
peroxide in an internal combustion engine which  
consists in introducing into the combustion  
chamber of the internal combustion engine a  
small proportion of an inorganic ferric com- 45  
pound.

ALFRED CHARLES GLYN EGERTON.